

June 4, 1974

SHOJI MARUYAMA ET AL  
6,6'-METHYLENEBIS[Z-STYRYL BENZOPYRYLIUM SALTS] AS  
SENSITIZERS FOR USE IN ELECTROPHOTOGRAPHIC  
LIGHT-SENSITIVE MATERIALS

3,814,752

Filed June 5, 1972

2 Sheets-Sheet 1

FIG. 1



FIG. 2



FIG. 3



FIG. 4



June 4, 1974

SHOJI MARUYAMA ET AL  
6,6'-METHYLENEBIS[ $\beta$ -STYRYL BENZOPYRYLIUM SALTS] AS  
SENSITIZERS FOR USE IN ELECTROPHOTOGRAPHIC  
LIGHT-SENSITIVE MATERIALS

3,814,752

Filed June 5, 1972

2 Sheets-Sheet 2



FIG. 6



FIG. 7



1

**3,814,752**  
**6,6'-METHYLENEBIS[2-STYRYL BENZOPYRYLIUM SALT] AS SENSITIZERS FOR USE IN ELECTROPHOTOGRAPHIC LIGHT-SENSITIVE MATERIALS**

Shoji Maruyama, Sagamihara, Kafue Kojima, Tomio Kubota, and Masahide Harada, Tokyo, and Masafumi Ohta, Yokohama, Japan, assignors to Ricoh Co., Ltd., Tokyo, Japan

Filed June 5, 1972, Ser. No. 259,392

Claims priority, application Japan, June 21, 1971, 46/44,739; July 7, 1971, 46/50,171

Int. Cl. C07d 7/46

U.S. Cl. 260—240 D

6 Claims

### ABSTRACT OF THE DISCLOSURE

There are provided sensitizers for use in an electrophotographic light-sensitive material containing an organic photoconductor. The sensitizers comprise derivatives of 6,6'-methylenebisbenzopyrylium salts.

### BACKGROUND OF THE INVENTION

It is well to use organic photoconductive materials such as polyvinylcarbazole instead of inorganic photoconductors such as photoconductive zinc oxide or selenium in electrophotographic light-sensitive materials. However, with organic photoconductors the sensitivity is low compared with inorganic photoconductors. Accordingly, in order to improve the sensitivity of organic photoconductors, it has been proposed to add certain coloring materials for sensitization. In this manner, the sensitivity of the organic photoconductive matter may be improved to a degree that it can be used in a practical manner. There is however still need for improvement.

It is an object of the present invention to provide sensitizers which will impart high sensitivity to organic photoconductors.

### SUMMARY OF THE INVENTION

The present invention relates to sensitizers for use in electrophotographic light-sensitive materials which contain organic photoconductors such as polyvinylcarbazole.

The sensitizers of the present invention are derivatives of 6,6'-methylenebisbenzopyrylium salts having the following general formula:



wherein R<sub>1</sub> is hydrogen, alkyl containing one to ten carbon atoms, or phenyl; R<sub>2</sub> is phenyl, naphthyl or styryl, or phenyl, naphthyl or styryl substituted with one to three alkoxy groups containing one to four carbon atoms; A<sup>-</sup> is ClO<sub>4</sub><sup>-</sup>, BF<sub>4</sub><sup>-</sup> or AuCl<sub>4</sub><sup>-</sup>.

Such derivatives of 6,6'-methylenebisbenzopyrylium salts have high sensitization effect on organic photoconductors. Furthermore, such derivatives have high molecular extinction coefficients and high thermal stability in comparison with benzopyrylium salts.

Typical derivatives of 6,6'-benzopyrylium salts used as a sensitizer in the present invention include:

Compound No. 1

6,6'-methylenebis[2-(2',3',4'-trimethoxystyryl)-3-phenylbenzopyrylium perchlorate]

Compound No. 2

6,6'-methylenebis[2-(4'-methoxynaphthylvinylene)-3-phenylbenzopyrylium perchlorate]

2

### Compound No. 3

6,6'-methylenebis[2-(3',4'-dimethoxystyryl)-3-phenylbenzopyrylium perchlorate]

Compound No. 4

6,6'-methylenebis[2-(p-methylstyryl)-3-phenylbenzopyrylium perchlorate]

Compound No. 5

10 6,6'-methylenebis[2-(2',4'-dimethoxystyryl)-3-phenylbenzopyrylium perchlorate]

Compound No. 6

15 6,6'-methylenebis[2-(p-methoxystyryl)-3-phenylbenzopyrylium perchlorate]

Compound No. 7

6,6'-methylenebis[2-(p-ethoxystyryl)-3-phenylbenzopyrylium perchlorate]

20 Compound No. 8

6,6'-methylenebis[2-(p-butoxystyryl)-3-phenylbenzopyrylium perchlorate]

Compound No. 9

25 6,6'-methylenebis[2-(p-methoxystyryl)benzopyrylium perchlorate]

Compound No. 10

30 6,6'-methylenebis[2-(p-methoxystyryl)-3-butylbenzopyrylium perchlorate]

Compound No. 11

35 6,6'-methylenebis[2-(p-ethoxystyryl)-3-octylbenzopyrylium perchlorate]

Compound No. 12

40 6,6'-methylenebis[2-(2',4'-dimethoxystyryl)-3-octylbenzopyrylium perchlorate]

Compound No. 13

45 6,6'-methylenebis[2-naphthylvinylene-3-phenylbenzopyrylium perchlorate]

Compound No. 15

50 6,6'-methylenebis[2-(3',4'-diethoxystyryl)-3-phenylbenzopyrylium perchlorate]

Such derivatives of 6,6'-methylenebisbenzopyrylium salts are used as sensitizers for an organic photoconductors such as polyvinylcarbazole or derivatives thereof. They are preferably used in an amount of 0.1 to 2.0% by weight based on the solid content, in a light-sensitive solution.

The effects of the sensitizers of the present invention are illustrated in the following examples.

### EXAMPLES 1-15

60 A light-sensitive solution was prepared as follows:

350 g. of a solution containing 6.7% brominated polyvinylcarbazole in chlorobenzene was mixed with 70 g. of a solution containing 10% polycarbonate in ethylene chloride and into this mixture was dissolved 4.7 g. of diphenyl chloride. To this solution was added a solution of the above sensitizers (Compound No. 1—No. 15) in dichloroethane. The sensitizers were used in the amount of 5×10<sup>-6</sup> mol of the sensitizer per 1 g. of brominated polyvinylcarbazole.

Electrophotographic light-sensitive materials were obtained by applying the light-sensitive solution to paper

and then drying. The light-sensitive solutions were applied so that the dried light-sensitive layer (coated layer) had a thickness of  $5\mu$  to  $6\mu$ .

After each light-sensitive product was allowed to stand in a dark place for several days, it was negatively charged by means of conventional corona discharge of 6 kv. and exposed to white light in contact with an image original while illuminating the surface of the light-sensitive layer at 20 lux.

In this manner, the optimum amount of exposure [lux-sec] required to obtain an exact reproduction of an original image on the light-sensitive layer was measured for each of Compounds No. 1 to No. 15.

Furthermore, by using the electrophotographic light-sensitive materials obtained above, the wave length of absorption maximum was measured by reflection method for each of Compounds No. 1 to No. 15.

The measured values are shown in the Table 1 below, and the curves of spectral sensitivity of the electrophotographic light-sensitive material sensitized with Compounds No. 1, No. 2 and No. 13 are shown in FIG. 1, FIG. 2 and FIG. 3 of the accompanying drawings, respectively.

TABLE 1

| Compound number | Optimum amount of exposure [lux-sec.] | Wave length of absorption maximum ( $\lambda_{max}$ ) [ $\mu$ ] |
|-----------------|---------------------------------------|-----------------------------------------------------------------|
| 1.....          | 38.5                                  | 614                                                             |
| 2.....          | 17.5                                  | 663                                                             |
| 3.....          | 47.5                                  | 610                                                             |
| 4.....          | 65.0                                  | 635                                                             |
| 5.....          | 33.0                                  | 590                                                             |
| 6.....          | 21.0                                  | 582                                                             |
| 7.....          | 37.5                                  | 590                                                             |
| 8.....          | 40.5                                  | 592                                                             |
| 9.....          | 85.5                                  | 580                                                             |
| 10.....         | 35.5                                  | 565                                                             |
| 11.....         | 33.0                                  | 580                                                             |
| 12.....         | 35.0                                  | 594                                                             |
| 13.....         | 36.6                                  | 566                                                             |
| 14.....         | 45.3                                  | 645                                                             |
| 15.....         | 36.5                                  | 585                                                             |

## EXAMPLES 16-30

Electrophotographic light-sensitive materials were obtained following the same procedures as that of Examples 1-15 except that chlorinated polyvinylcarbazole was employed as a substitute for brominated polyvinylcarbazole.

The electrophotographic light-sensitive materials yielded an exact reproduction of original images in the same manner as that of Examples 1-15 except that the light-sensitive materials were exposed to light for 2 seconds while illuminating the surface of the light-sensitive layer at 20 lux.

Derivatives of 6,6'-methylenebisbenzopyrylium salts having general formula (I) are synthesized as follows:

Condensation of 5,5'-methylenebissalicylaldehyde of formula (II) with a ketone of general formula (III) is carried out and to this reaction solution is added an aldehyde of general formula (IV) to carry out cyclic condensation.



In the equation  $R_1$  and  $R_2$  are the same groups as in the general formula (I).

5,5'-methylenebissalicylaldehyde (II), ketone (III) and aldehyde (IV) may be synthesized by conventional method.

The condensation and cyclic condensation are carried out in a solvent. As a solvent for 5,5'-methylenebissalicylaldehyde (II), tetrahydrofuran, alcohols and ether may be used. As a solvent for ketone (III) and aldehyde (IV), an organic acid such as formic acid or acetic acid may be used.

As a condensing agent for the condensation and the cyclic condensation, hydrochloric acid or hydrogen chloride may be used.

The reaction temperature of the condensation and the cyclic condensation is preferably between 0° C. and 5° C.

Introduction of an anion is effected as follows:

(1) After the cyclic condensation with aldehyde has been carried out in the presence of acid or salt having the desired anion, the reaction solution is poured into ether to crystallize.

(2) After cyclic condensation has been carried out, the reaction solution is poured into a cooled solution (concentration: 5-20%) containing acid or salt having a desired anion to crystallize.

Methods of producing derivatives of 6,6'-methylenebisbenzopyrylium salt are illustrated by the following Preparations No. 1 to No. 5.

## Preparation No. 1

6,6'-methylenebis[2-(p-methoxystyryl)-3-phenylbenzopyrylium perchlorate] (Compound No. 6 having the following formula)



2.5 g. of 5,5'-methylenebissalicylaldehyde was dissolved in 40 ml. of tetrahydrofuran and to this solution was added a solution containing 3 g. of benzyl methyl ketone in 20 ml. of 90% formic acid. After having been well mixed, the solution was saturated with hydrogen chloride while cooling. The solution was allowed to stand in an ice box for 2 hours and then to this solution was added a solution containing 3 g. of p-methoxybenzaldehyde in 20 ml. of 90% formic acid. After this solution was saturated with hydrogen chloride while cooling and allowed to stand in an ice box for 2 days, the solution was poured into a 15% cooled aqueous solution of perchloric acid ( $\text{HClO}_4$ ). Crude crystals separated from the solution by allowing to stand for 30 minutes were filtered and recrystallized from 300 ml. of 90% acetic acid. 9.3 g. of crystals of the captioned compound (M.P. 185° C-187° C.) was thus obtained.

| 50              | Analysis (for $\text{C}_{40}\text{H}_{38}\text{Cl}_2\text{O}_{12}$ ) | Percent of— |      |      |
|-----------------|----------------------------------------------------------------------|-------------|------|------|
|                 |                                                                      | C           | H    | Cl   |
| Calculated..... |                                                                      | 66.21       | 4.27 | 7.88 |
| Found.....      |                                                                      | 66.12       | 4.18 | 8.05 |

55 This compound showed wave length of absorption maximum ( $\lambda_{max}$ ) at 576  $\mu$  and molecular extinction coefficient ( $\epsilon$ ) of  $10.76 \times 10^4$  in dichloroethane.

## Preparation No. 2

60 6,6'-methylenebis[2-(4'-methoxynaphthylvinylene)-3-phenylbenzopyrylium perchlorate] (Compound No. 2 having the following formula)



70 2.5 g. of 5,5'-methylenebissalicylaldehyde was dissolved in 40 ml. of tetrahydrofuran and to this solution was added a solution containing 3 g. of benzyl methyl ketone in 20 ml. of 90% formic acid. After having been well mixed, this solution was saturated with hydrogen chloride while cooling. The solution was allowed to stand in an ice box for 2 hours and then to this solution was added a

5  
solution containing 4 g. of 4-methoxynaphthaldehyde in 20 ml. of 90% formic acid. This solution was saturated with hydrogen chloride while cooling and thereafter the same procedure as that of Preparation No. 1 was repeated. 7.7 g. of crystals of the captioned compound (M.P. 228° C.-229° C.) was thus obtained.

| Percent of—                                                                     |       |      |
|---------------------------------------------------------------------------------|-------|------|
| Analysis (for C <sub>37</sub> H <sub>12</sub> Cl <sub>2</sub> O <sub>12</sub> ) | C     | H    |
| Calculated.....                                                                 | 69.23 | 4.25 |
| Found.....                                                                      | 69.18 | 4.14 |
|                                                                                 |       | 7.08 |
|                                                                                 |       | 6.88 |

This compound showed wave length of absorption maximum  $\lambda_{\text{max}}$  at 660 m $\mu$  and molecular extinction coefficient ( $\epsilon$ ) of  $8.7 \times 10^4$  in dichloroethane. Infrared absorption spectrum and transmission absorption spectrum of this compound are respectively shown in FIG. 4 and FIG. 6 of the accompanying drawings.

#### Preparation No. 3

6,6'-methylenebis[2 - (p - methoxystyryl) - 3 - decylbenzopyrylium-perchlorate] (Compound No. 13 having the following formula)



5 g. of 5,5'-methylenebissalicylaldehyde was dissolved in 50 ml. of ethyl alcohol and to this solution was added a solution containing 7.6 g. of methyl undecyl ketone in 40 ml. of 90% acetic acid. After having been well mixed, the solution was saturated with hydrogen chloride while cooling. The solution was allowed to stand in an ice box for 4 days and then to this solution was added a solution containing 5.2 g. of p-methoxybenzaldehyde in 20 ml. of 90% formic acid. This solution was saturated with hydrogen chloride, and thereafter the same procedure as that of Preparation No. 1 was repeated. 13.5 g. of crystals of the captioned compound (M.P. 173° C.-174° %C.) was thus obtained.

| Percent of—                                                                     |       |      |
|---------------------------------------------------------------------------------|-------|------|
| Analysis (for C <sub>37</sub> H <sub>70</sub> Cl <sub>1</sub> O <sub>12</sub> ) | C     | H    |
| Calculated.....                                                                 | 62.40 | 6.38 |
| Found.....                                                                      | 62.33 | 6.42 |
|                                                                                 |       | 6.38 |
|                                                                                 |       | 6.35 |

This compound showed wave length of absorption maximum ( $\lambda_{\text{max}}$ ) at 559 m $\mu$  and molecular extinction coefficient ( $\epsilon$ ) of  $8.79 \times 10^4$  in dichloroethane.

#### Preparation No. 4

6,6' - methylenebis[2 - (2',3',4' - trimethoxystyryl)-3-phenylbenzopyrylium perchlorate] (Compound No. 1 having the following formula)



2.5 g. of 5,5'-methylenebissalicylaldehyde was dissolved in 40 ml. of tetrahydrofuran and to this solution was added a solution containing 3 g. of benzyl methyl ketone in 20 ml. of 90% acetic acid. After having been well mixed, the solution was saturated with hydrogen chloride while cooling. The solution was allowed to stand in an ice box for 2 hours and then to this solution was added a solution containing 4 g. of 2,3,4-trimethoxybenzaldehyde in 30 ml. of 90% acetic acid. This solution was saturated with hydrogen chloride while cooling and thereafter the same procedure as that of Preparation No. 1 was repeated

6  
8.0 g. of crystals of the captioned compound (M.P. 223° C.-225° C.) was thus obtained.

| Percent of—                                                                     |       |      |
|---------------------------------------------------------------------------------|-------|------|
| Analysis (for C <sub>33</sub> H <sub>14</sub> Cl <sub>2</sub> O <sub>10</sub> ) | C     | H    |
| Calculated.....                                                                 | 63.09 | 4.56 |
| Found.....                                                                      | 62.72 | 4.47 |
|                                                                                 |       | 6.94 |
|                                                                                 |       | 7.14 |

10 This compound showed wave length of absorption maximum  $\lambda_{\text{max}}$  at 607 m $\mu$  and molecular extinction coefficient ( $\epsilon$ ) of  $7.4 \times 10^4$  in dichloroethane.

#### Preparation No. 5

15 6,6'-methylenebis[2 - (2',4' - dimethoxystyryl)-3-octylbenzopyrylium perchlorate] (Compound No. 12 having the following formula)



20 2.6 g. of 5,5'-methylenebissalicylaldehyde was dissolved in 50 ml. of tetrahydrofuran and to this solution was added a solution containing 3.4 g. of methyl nonyl ketone in 20 ml. of 90% formic acid. After having been well mixed, the solution was saturated with hydrogen chloride while cooling. The solution was allowed to stand in an ice box for 3 days and then to this solution was added a solution containing 3.2 g. of 2,4-dimethoxybenzaldehyde in 10 ml. of 90% formic acid. This solution was saturated with hydrogen chloride while cooling and thereafter the same procedure as that of Preparation No. 1 was repeated. 7.5 g. of crystals of the captioned compound (M.P. 200° C.;202° C.) was thus obtained.

| Percent of—                                                                     |       |      |
|---------------------------------------------------------------------------------|-------|------|
| Analysis (for C <sub>68</sub> H <sub>25</sub> Cl <sub>2</sub> O <sub>14</sub> ) | C     | H    |
| Calculated.....                                                                 | 64.57 | 6.45 |
| Found.....                                                                      | 64.38 | 6.51 |
|                                                                                 |       | 6.84 |
|                                                                                 |       | 6.90 |

45 This compound showed wave length of absorption maximum ( $\lambda_{\text{max}}$ ) at 587 m $\mu$  and molecular extinction coefficient ( $\epsilon$ ) of  $6.53 \times 10^4$  in dichloroethane. Infrared absorption spectrum and transmission absorption spectrum of this compound are respectively shown in FIG. 5 and FIG. 7 of the accompanying drawings.

50 The following derivatives of 6,6'-methylenebisbenzopyrylium salt could be obtained by repeating the same procedure as that mentioned above except that suitable aldehyde and ketone were used.

55 6,6'-methylenebis[2-naphthylvinylene-3-phenylbenzopyrylium perchlorate] (Compound No. 14)



(M.P. 218° C.-220° C.)

60 6,6'-methylenebis[2-(p-methoxystyryl)-3-butylbenzopyrylium perchlorate] (Compound No. 10)



(M.P. 249° C.-251° C.)

6,6'-methylenabis[2-(3',4'-dimethoxystyryl)-3-phenylbenzopyrylium perchlorate] (Compound No. 3)



(M.P. 249° C.-250° C.)

6,6'-methylenabis[2-(p-ethoxystyryl)-3-phenylbenzopyrylium perchlorate] (Compound No. 7)



(M.P. 250° C.-251° C.)

In the above-mentioned Examples and Preparations, benzopyrylium salts having  $\text{ClO}_4^-$  as an anion have been shown. Benzopyrylium salts having  $\text{BF}_4^-$  or  $\text{AuCl}_4^-$  as an anion can be obtained by using an aqueous solution of sodium tetrafluoroborate ( $\text{NaBF}_4$ ) or chloroauric acid ( $\text{HAuCl}_4$ ) instead of an aqueous solution of perchloric acid ( $\text{HClO}_4$ ).

We claim:

1. A sensitizer for use in an electrophotographic light-sensitive material having the formula (I):



wherein  $R_1$  is hydrogen, alkyl containing one to ten carbon atoms, or phenyl;  $R_2$  is phenyl, naphthyl or styryl or phenyl, naphthyl or styryl substituted with one to three alkoxy groups containing one to four carbon atoms;  $A^-$  is  $\text{ClO}_4^-$ ,  $\text{BF}_4^-$  or  $\text{AuCl}_4^-$ .

2. A sensitizer according to claim 1 wherein the derivative is 6,6'-methylenabis[2-(p-methoxystyryl)-3-phenylbenzopyrylium perchlorate].

3. A sensitizer according to claim 1 wherein the derivative is 6,6'-methylenabis[2-(4-methoxynaphthylvinylene)-3-phenylbenzopyrylium perchlorate].

4. A sensitizer according to claim 1 wherein the derivative is 6,6'-methylenabis[2-(p-methoxystyryl)-3-decylbenzopyrylium perchlorate].

5. A sensitizer according to claim 1 wherein the derivative is 6,6'-methylenabis[2-(2',3',4'-trimethoxystyryl)-3-phenylbenzopyrylium perchlorate].

6. A sensitizer according to claim 1 wherein the derivative is 6,6'-methylenabis[2-(2',4'-dimethoxystyryl)-3-octylbenzopyrylium perchlorate].

#### References Cited

#### FOREIGN PATENTS

22,748 7/1970 - Japan 260-240 D

JOHN D. RANDOLPH, Primary Examiner

S. D. WINTERS, Assistant Examiner

#### U.S. CL. X.R.

260-240 R, 600; 96-1.6